

2,765,269

## BATH FOR PLATING BRIGHT GOLD

Barnet D. Ostrow, North Bellmore, and Fred I. Nobel,  
North Valley Stream, N. Y.

No Drawing. Application November 19, 1954,  
Serial No. 470,136

7 Claims. (Cl. 204—46)

The present invention is directed to electroplating baths, more particularly to a gold cyanide plating bath adapted to produce bright deposits which do not require brushing or buffing.

Gold plating baths capable of producing bright deposits have been known and used. The degree of brightness obtained by such baths has been about equivalent to the brightness obtained by the use of present day bright nickel baths. However, such bright gold baths required certain special equipment of a highly specialized character in order to obtain the optimum results in the operation. Such equipment required close attention and a high degree of skill on the part of the operator. Therefore there has been a need for a bath which was adapted to give bright gold deposits without the necessity of special equipment or special attention on the part of the operator.

The present invention is intended and adapted to overcome the disadvantages inherent in prior bright gold baths, it being among the objects of the present invention to provide a bath which is capable of reproducing in the gold deposit the brightness present in the basis metal.

It is also among the objects of the present invention to provide a bath giving a bright gold deposit which requires no scratch brushing or coloring.

It is further among the objects of the present invention to provide a bath of the character described, which is simple in operation, which is easy to control and which is capable of providing optimum operating results.

In practicing the present invention there is provided a cyanide bath of well-known character consisting essentially of gold cyanide and free alkali metal cyanide in solution with water. In accordance with the invention, there is added to the bath two types of substances, one of which is a condensation product of certain carboxylic acids and certain amino acids. There is also present in the bath in relatively small amount a soluble nickel salt and/or a soluble tin salt. The invention also contemplates the presence at the same time of both nickel and tin salts.

The condensation product is made by reacting a fatty acid having from 8 to 18 carbon atoms with an amino acid. The resulting condensation product is believed to have the following structural formula:



wherein M represents hydrogen and alkali metal, R represents an alkyl radical having 7 to 17 carbon atoms, R' represents a lower fatty acid, an alkyl monoalcohol, ester thereof, ether thereof, the alkyl radicals of which have 1 to 3 carbon atoms and hydrogen, and R'' represents methylene, ethylene and propylene, together with a water soluble salt of a metal taken from the class consisting of nickel and/or tin. The amount of said condensation product ranges from 1 to 100 grams per liter and good results are obtained by the use of 25-30 grams per liter in the bath.

The nickel may be present in the form of any soluble salt thereof which does not interfere with the plating operation, such as the sulphate, cyanide and the like, the amount of nickel present in the bath ranging from 0.10 to 50 grams per liter. Any such salt will upon addition to the bath form complex alkali metal cyanide. The tin is also present as a soluble compound and it has been found that an excellent form is that of alkali metal stannates, the amount of tin present in the bath ranging from 0.01 to 20 grams per liter. Mixtures of salts of this character may be added to the bath.

The following are specific examples showing a number of baths which are suitable for the present purposes. The formulas of the following examples show the relative amounts of the constituents in grams per liter. Electroplating takes place at temperatures between 70° and 90° F. with vigorous agitation for the best results. The current densities range from 0 to 20 amperes per square foot, depending on the gold concentration.

20 *Example 1*

|                                            |      |
|--------------------------------------------|------|
| Gold as KAu cyanide                        | 7.5  |
| Nickel as K <sub>2</sub> Ni cyanide        | 3.0  |
| Potassium stannate                         | 4.0  |
| 25 Free potassium cyanide                  | 80.0 |
| N-methylglycine-lauric acid potassium salt | 20.0 |

*Example 2*

|                                            |      |
|--------------------------------------------|------|
| Gold as KAu cyanide                        | 10.0 |
| 30 Potassium stannate                      | 6.0  |
| Free potassium cyanide                     | 90.0 |
| N-ethanolglycine-myristic acid sodium salt | 30.0 |

*Example 3*

|                                           |      |
|-------------------------------------------|------|
| 35 Gold as KAu cyanide                    | 4.5  |
| Nickel as Ni sulphate                     | 20.0 |
| Free potassium cyanide                    | 15.0 |
| N-acetylglycine-myristic acid-sodium salt | 25.0 |

*Example 4*

|                                       |      |
|---------------------------------------|------|
| 40 Gold as KAu cyanide                | 5.5  |
| Nickel as K <sub>2</sub> Ni cyanide   | 3.5  |
| Free potassium cyanide                | 20.0 |
| N-ethylglycine-oleic acid sodium salt | 35.0 |

*Example 5*

|                                                    |      |
|----------------------------------------------------|------|
| Gold as NaAu cyanide                               | 9.0  |
| Sodium stannate                                    | 5.5  |
| Free sodium cyanide                                | 25.0 |
| 50 N-methylmethyleglycine-stearic acid sodium salt | 20.0 |

Methods of making the condensation products of the fatty acids and amino acids are well-known.

Such compounds made from sarcosine have been mentioned in the prior art for use in silver cyanide plating baths. However, gold deposits obtained from gold cyanide plating baths containing such condensation products, are not bright when the bath contains only these complex condensation products as brighteners. It is only when there is present in the bath in addition thereto 60 of a soluble compound of tin or nickel, or a mixture of such compounds of the two metals, that bright gold deposits can be obtained. And the optimum brightness of such deposits are obtained when both tin and nickel are present together with the organic condensation product.

65 Such a combination has an important advantage in connection with the operation of the bath. The presence of the condensation product increases substantially the tolerance of the plating bath for organic impurities and contamination. While in the prior art it had been suggested to use other precious metals for the purpose of producing bright gold deposits, such additions increase costs to a substantial extent and furthermore, are not as bright.

become very sensitive to organic contamination. The present composition effectively eliminates these difficulties.

We claim:

1. In a bright gold plating bath consisting essentially of gold cyanide and free alkali metal cyanide in water solution, the improvement which comprises the addition to said bath of a condensation product of a fatty acid having 8 to 18 carbon atoms with an amino acid and having the following structural formula:



wherein M represents a radical taken from the class consisting of hydrogen and alkali metal, R represents an alkyl radical having 7 to 17 carbon atoms, R' represents a radical taken from the class consisting of a lower fatty acid, an alkyl monoalcohol, ester thereof, ether thereof, the alkyl radicals of which have 1 to 3 carbon atoms and hydrogen, and R'' represents a radical taken from the class consisting of methylene, ethylene and propylene, the amount of said reaction product being from 1 to 100 gms./liter, together with the water soluble salts of nickel and tin in sufficient amount to exert a brightening effect on the plated gold.

2. In a bright gold plating bath consisting essentially of gold cyanide and free alkali metal cyanide in water solution, the improvement which comprises the addition of said bath of a condensation product of a fatty acid having 8 to 18 carbon atoms with an amino acid and having the following structural formula:



wherein M represents a radical taken from the class consisting of hydrogen and alkali metal, R represents an alkyl radical having 7 to 17 carbon atoms, R' represents a radical taken from the class consisting of a lower fatty acid, an alkyl monoalcohol, ester thereof, ether thereof, the alkyl radicals of which have 1 to 3 carbon atoms and hydrogen, and R'' represents a radical taken from the class consisting of methylene, ethylene and propylene, the amount of said reaction product being about 25-30 gms./liter, together with the water-soluble salts of nickel and tin in sufficient amount to exert a brightening effect on the plated gold.

3. In a bright gold plating bath consisting essentially of gold cyanide and free alkali metal cyanide in water solution, the improvement which comprises the addition to said bath of a condensation product of a fatty acid having 8 to 18 carbon atoms with an amino acid and having the following structural formula:



wherein M represents a radical taken from the class consisting of hydrogen and alkali metal, R represents an alkyl radical having 7 to 17 carbon atoms, R' represents a radical taken from the class consisting of a lower fatty acid, an alkyl monoalcohol, ester thereof, ether thereof, the alkyl radicals of which have 1 to 3 carbon atoms and hydrogen, and R'' represents a radical taken from the class consisting of methylene, ethylene and propylene, the amount of said reaction product being about 1-100 grams per liter, together with the water-soluble salts of nickel and tin, the amount of nickel being from 0.1 to 50

gms./liter and the amount of tin being from 0.01 to 20 gms./liter.

4. In a bright gold plating bath consisting essentially of gold cyanide and free alkali metal cyanide in water solution, the improvement which comprises the addition to said bath of the following composition in grams per liter:

|                                              |         |
|----------------------------------------------|---------|
| Tin as alkali metal stannate                 | 0.01-20 |
| Nickel as soluble nickel salt                | 0.10-50 |
| Condensation product of fatty and amino acid | 1-100   |

said tin and nickel being present in sufficient amount to exert a brightening effect, said condensation product having the following structural formula:



wherein M represents a radical taken from the class consisting of hydrogen and alkali metal, R represents an alkyl radical having 7 to 17 carbon atoms, R' represents a radical taken from the class consisting of a lower fatty acid, an alkyl monoalcohol, ester thereof, ether thereof, the alkyl radicals of which have 1 to 3 carbon atoms and hydrogen, and R'' represents a radical taken from the class consisting of methylene, ethylene and propylene.

5. In a bright gold plating bath consisting essentially of gold cyanide and free alkali metal cyanide in water solution, the improvement which comprises the addition to said bath of the following composition in grams per liter:

|                                              |         |
|----------------------------------------------|---------|
| Tin as alkali metal stannate                 | 0.01-20 |
| Nickel as soluble nickel salt                | 0.10-50 |
| Condensation product of fatty and amino acid | 1-100   |

said tin and nickel being present in sufficient amount to exert a brightening effect, said condensation product being of N-methyl glycine with an acid taken from the class consisting of oleic, stearic, palmitic, lauric and myristic.

6. In a bright gold plating bath consisting essentially of gold cyanide and free alkali metal cyanide in water solution, the improvement which comprises the addition to said bath of the following composition in grams per liter:

|                                              |         |
|----------------------------------------------|---------|
| Tin as alkali metal stannate                 | 0.01-20 |
| Nickel as soluble nickel salt                | 0.10-50 |
| Condensation product of fatty and amino acid | 1-100   |

said tin and nickel being present in sufficient amount to exert a brightening effect, said condensation product being of N-methyl glycine with the mixed acids of coconut type oil.

7. A bath according to claim 1 in which the amino acid is a glycine.

#### References Cited in the file of this patent

#### FOREIGN PATENTS

1,027,637 France Feb. 18, 1953

#### OTHER REFERENCES

Serial No. 351,241, Weiner (A. P. C.), published May 18, 1943.